

## UNITED STATES PATENT OFFICE

2,002,406

## PROCESS OF DYEING

Robert Lantz, Paris, France, assignor of one-half to Societe Anonyme des Matieres Colorantes & Produits Chimiques de Saint-Denis, Paris, France

No Drawing. Application June 11, 1931, Serial No. 543,730. In France June 21, 1930

10 Claims. (Cl. 8—5)

Although azo-dyestuffs containing a disulphide or trisulphide group in the molecule have already been described, the use of these dyestuffs for dyeing in a sulphide bath has involved difficulties 5 which do not appear to have been overcome. In particular the dyeings obtained on cotton are generally weak and the dyestuffs appear to have no affinity for the material.

This invention is based on the discovery that 10 these difficulties are due to the fact that the dyestuffs are destroyed by the sulphide bath at a temperature which is generally lower than that commonly used in practice in dyeing with sulphur dyestuffs. It is probable that the azo-linkage undergoes reduction by the sulphide which itself becomes oxidized; the quantity of sulphide in the bath, therefore, decreases and may become insufficient for maintaining the unattacked dyestuff in solution. In consequence it is difficult to 15 obtain satisfactory dyeings. It may be noted that this behaviour is unexpected for it is known that sulphides in general are not capable of reducing an azo-linkage (Lange, "Die Schwefelfarbstoffe", 2nd edn. page 69).

According to the invention the difficulties in 20 dyeing in a sulphide bath with azo-dyestuffs containing a disulphide or trisulphide group in the molecule are overcome by conducting the dyeing at a relatively low temperature. These dyestuffs may be made either according to known 25 processes or by the process described in my U. S. patent application Ser. No. 543,746 filed June 11, 1931 which consists in coupling tetrazotized 4:4'-diaminodiphenyl-disulphide with an azo-component with the exception of  $\beta$ -naphthylamine, or again by the process described in my U. S. patent application Ser. No. 543,747 filed June 11, 1931, which consists in coupling the diazo-compound of an ortho-aminophenol with an azo compound 30 containing at least one di- or trisulphide group in the molecule. It has been found unexpectedly that the majority of these dyestuffs have a good affinity for vegetable fibres and regenerated cellulose fibres, so much so that in many cases it is possible to obtain full dyeings even at ordinary 35 temperature. For example, the dyestuff made in the manner described in German Specification No. 161,462 by coupling tetrazotized 4:4'-diamino-2:2'-dinitrodiphenylsulphide with  $\beta$ -naphthol yields an intense orange shade when dyeing is conducted at ordinary temperature, whilst when dyeing is conducted in the manner usual in the case of sulphur dyestuffs, there is obtained a weak bluish-red shade described in the aforesaid Ger-

man specification. However, the latter shade may also be obtained, but in greater depth, when dyeing is conducted at ordinary temperature, if the dyestuff is allowed to remain for a long time in solution in presence of a sulphide either before or during the dyeing operation. 5

The most favourable temperature is generally in the neighbourhood of atmospheric temperature; it may, however, be advantageous to work at a higher temperature. According to the depth 10 of dyeing required there may be added to the dye-bath in greater or lesser quantity a neutral electrolyte, such as sodium sulphate or sodium chloride. In particular cases it may be advantageous to render the dye-bath more alkaline by 15 the addition of a small proportion of caustic soda or sodium carbonate, or less alkaline by the addition, for example, of sodium hydrosulphide or sodium bicarbonate.

The invention is applicable not only for dyeing 20 vegetable fibres but for dyeing fibres of regenerated cellulose or of cellulose ethers or cellulose esters.

The dyeings may subsequently be subjected to 25 oxidation or to a treatment which is customary after dyeing or to more than one of these operations.

The depth of the dyeings may be increased or 30 their shade altered by subjecting the dyed goods to one or more repetitions of the process either using the same dyestuff or a different dyestuff.

The following examples illustrate the invention the parts being by weight unless otherwise stated: 35

*Example 1.*—One part of the dyestuff made by combining tetrazotized 2:2'-dinitro-4:4'-diaminodiphenylsulphide with  $\beta$ -naphthol (see German specification No. 161,462) is dissolved at ordinary temperature in 5 parts by volume of 40 a solution containing 2 parts of crystallized sodium sulphide and the solution is diluted by the addition of 150 parts by volume of a solution containing 22.5 parts of crystallized sodium sulphate. 10 parts of cotton are introduced into the 45 bath and maintained in motion therein during one hour at ordinary temperature. The material is then washed and subjected to oxidation, for example by means of a dilute solution by hydrogen peroxide. A full orange shade is obtained whereas if cotton is dyed in the hitherto usual manner with the same dyestuff only a weak bluish-red shade is obtained. 50

In like manner dyeing may be conducted with

satisfactory results with the dyestuffs indicated *Example 3.*—50.5 parts of the dyestuff obtained by coupling tetrazotized para:para'-di-

| Dyestuff                                                      |                                                         | Colour of dyeing on cotton, after oxidation | 5  |
|---------------------------------------------------------------|---------------------------------------------------------|---------------------------------------------|----|
| 5                                                             | Tetrazo-compound of—                                    | Coupled with 2 molecular proportions of—    |    |
| 2:2'-dinitro-4:4'-diamino-diphenyldisulphide                  | Meta-phenylenediamine                                   | Brown-yellow.                               |    |
| Do                                                            | $\beta$ -naphthol                                       | Orange.                                     |    |
| Do                                                            | 2:7-dihydroxynaphthalene                                | Brown-orange.                               | 10 |
| 10 4:4'-diaminodiphenyldisulphide (para-para'-dithioaniline)  | Phenylmethylpyrazolone                                  | Yellow.                                     |    |
| Do                                                            | $\beta$ -naphthol                                       | Vivid yellowish-red.                        |    |
| Do                                                            | $\alpha$ -naphthol                                      | Brown-purple.                               |    |
| Do                                                            | 2:7-dihydroxynaphthalene                                | Brown.                                      |    |
| Do                                                            | Meta-phenylenediamine                                   | Brown-yellow.                               |    |
| 15 4:4'-diaminodiphenyl disulphide (para-para'-dithioaniline) | $\beta$ -oxynaphthoic acid-para:para'-dithioaniline     | Bluish-red.                                 | 15 |
| Do                                                            | Bis(2 hydroxynaphthyl 6) disulphide                     | Red.                                        |    |
| Do                                                            | Trisulphide of $\alpha$ -naphthol                       | Red-purple.                                 |    |
| Aniline                                                       | $\beta$ -hydroxynaphthoic acid-para:para'-dithioaniline | Red.                                        |    |

The conditions indicated in the foregoing example may be varied within wide limits. The dyestuff may be used in a different concentration, the concentration of sodium sulphate or other metal salt may be increased or reduced. There may be added to the dye-bath a neutralizing agent, such as sodium bicarbonate or sodium hydrosulphide, or an agent which renders the bath more alkaline, such as sodium carbonate or caustic soda. There may also be used any of the various additions usual in dyeing, such as glue, sulphonated oils and other substances adapted to improve the penetration of the fibre or to hinder the precipitation of the dyestuff. The dyeing may be oxidized by means of atmospheric oxygen, a very dilute solution of sodium hypochlorite, ferric chloride or the like.

35 In the case of certain dyestuffs the dissolution or the dyeing operation may be conducted at a higher temperature which must, however, be lower than that at which the dyestuff is destroyed or altered.

40 *Example 2.*—One part of the dyestuff obtained by coupling diazotized 4-chloro-2-amino-1-phenol with  $\beta$ -hydroxy-naphthoic acid para:para'-dithioaniline (compare Example 3 of French patent application No 297,526 filed June 20, 1930) is dissolved in 2 parts of caustic soda solution of 36° Bé. and 5 parts of a solution containing 2 parts of crystallized sodium sulphide and there are then added 170 parts by volume of a solution containing 50 parts of crystallized sodium sulphate. 10 parts of cotton are dyed by immersion for 50 minutes at ordinary temperature in the dye-bath so prepared. By oxidation of the dyeing, for example by means of dilute hydrogen peroxide or air, there is obtained a bluish-red shade. By subsequent treatment of the dyeing with a solution of a copper salt, such as copper sulphate, and acetic acid there is obtained a violet shade of remarkable fastness to light. As in the preceding example the conditions of dyeing may be substantially modified.

55 The properties of a number of dyeings obtainable by the invention and after treated with metal salts are indicated in the following table:

| 65                      | Dyestuff                                     | Treated with a salt of— | Shade         | 65 |
|-------------------------|----------------------------------------------|-------------------------|---------------|----|
|                         | Diazo- or tetrazo- component                 | Coupled with—           |               |    |
| 70 Dithioaniline        | $\beta$ -naphthol                            | Chromium                | Vivid red.    |    |
| Dithioaniline           | $\beta$ -naphthol                            | Copper                  | Brownish-red. | 70 |
| Nitro-orthoaminophenol  | $\beta$ -hydroxynaphthoic acid-dithioaniline | Copper                  | Bordeaux.     |    |
| Chloro-orthoaminophenol | $\beta$ -hydroxynaphthoic acid-dithioaniline | Copper                  | Violet-red.   |    |
| Picramic acid           | $\beta$ -hydroxynaphthoic acid-dithioaniline | Copper                  | Dark violet.  |    |
| Ortho-aminophenol       | Bis(2 hydroxynaphthyl 6) disulphide          | Copper                  | Bordeaux.     |    |
| Nitro-orthoaminophenol  | Bis(2 hydroxynaphthyl 6) disulphide          | Copper                  | Violet.       |    |
| Chloro-orthoaminophenol | Trisulphide of $\alpha$ -naphthol            | Copper                  | Brown-red.    |    |

75

thioaniline with  $\alpha$ -naphthylamine (compare Example 2 of U. S. patent application Ser. No. 543,746 filed June 11, 1931) are dissolved in 25 parts by volume of a solution containing 10 parts of crystallized sodium sulphide and there are then added 375 parts by volume of a cold solution containing 112 parts of crystallized sodium sulphate. 25 parts of cotton are dyed for 30 minutes at ordinary temperature in the bath so prepared. After oxidation a brown dyeing is obtained. It may be diazotized in the usual manner in a bath containing nitrous acid and then introduced into a feebly alkaline bath containing  $\beta$ -naphthol; a black shade is thus obtained. The diazotized dyeing may of course be coupled with other azodye-stuff coupling components.

35 *Example 4.*—The procedure is as described in Example 1 with the exception that instead of adding the solution of sodium sulphate immediately after dissolution of the dyestuff, the solution of the dyestuff is first allowed to stand for 3 hours. The dyeing thus obtained, instead of being orange, is red.

40 *Example 5.*—Cellulose regenerated from viscose is dyed in the manner indicated in Example 1 with the dyestuff from tetrazotized para:para'-dithioaniline and  $\beta$ -naphthol. The shade is fuller and its fastness to light greater than in the case of the dyeing on cotton.

45 *Example 6.*—Artificial silk of acetyl cellulose is dyed in the manner indicated in Example 1, the duration of the dyeing operation, however, being increased to 2 hours. There is obtained a very vivid orange-red shade, without alteration of the silk.

50 A bluish-red shade is obtained by using the dyestuff from tetrazotized dithioaniline and  $\beta$ -hydroxynaphthoic acid dithioaniline.

55 *Example 7.*—Cotton is dyed in the manner indicated in Example 1 with the dyestuff from tetrazotized dithioaniline and  $\beta$ -naphthol. After oxidation of the dyeing by means of air or hydrogen peroxide, the dyed cotton is re-introduced into the same dye-bath and dyed in the same manner as before. The depth of the red dyeing

is thus increased. The dyeing operation may be repeated several times.

*Example 8.*—The fibre which has been dyed red in the manner described in Example 1 by means of the dyestuff from tetrazotized para:para'-dithioaniline and  $\beta$ -naphthol, is introduced after the oxidation into a second dye-bath prepared in the same manner with the dyestuff from tetrazotized para:para'-dithioaniline and methyl-phenylpyrazolone (Example 1 of U. S. patent application Ser. No. 543,746 filed June 11, 1931). An orange red shade is thus obtained.

What I claim is:

1. A process of dyeing materials which comprises treating said materials in a sulphide bath by an azo-dyestuff containing at least one disulphide group in the molecule at a temperature lower than 65° C.

2. A process of dyeing materials which comprises taking the dyestuff resulting from the coupling of the tetrazo compound of 4:4'-diaminodiphenyldisulphide (para - para' - dithioaniline) with meta-phenylenediamine, dissolving it at a temperature lower than 65° C. in a solution of crystallized sodium sulphide, adding a solution containing sodium sulphate, introducing the material to be treated into the bath thus obtained, allowing it to remain therein for a certain time, washing it and oxidizing it.

3. A process of dyeing materials which comprises taking the dyestuff resulting from the coupling of the tetrazo compound of 4:4'-diaminodiphenyldisulphide (para-para'-dithioaniline) with  $\beta$ -hydroxynaphthoic acid - para:para'-dithioaniline, dissolving it at a temperature lower than 65° C. in a solution of crystallized sodium sulphide, adding a solution containing crystallized sodium sulphate, introducing the material to be treated into the bath thus prepared, allowing it to remain therein for a certain time, washing it and oxidizing it.

4. A process of dyeing materials which comprises taking the dyestuff resulting from the coupling of the tetrazo compound of 4:4'-diaminodiphenyldisulphide (para-para'-dithioaniline) with bis (2 hydroxynaphthyl 6) disulphide dissolving said dyestuff at a temperature lower than 65°

C. in a solution of crystallized sodium sulphide, adding a solution containing crystallized sodium sulphate, introducing the material to be treated into the bath thus obtained, allowing it to remain therein for a certain time, washing it and oxidizing it.

5. A process of dyeing materials which comprises taking the dyestuff resulting from the coupling of an azo-compound of nitro-orthoamino-phenol with  $\beta$ -hydroxynaphthoic acid-dithioaniline, dissolving it at a temperature lower than 65° C. in a bath containing a caustic soda solution, and a solution of crystallized sodium sulphide, adding a solution of crystallized sodium sulphate, immersing into the bath thus obtained the material to be treated, and oxidizing the dyed material.

6. A process of dyeing materials which comprises treating said materials in a sulphide bath by an azo-dyestuff containing at least one disulphide group in the molecule, at a temperature lower than 65° C., oxidizing the dyed material and treating it with another dye-bath.

7. A process of dyeing materials which comprises treating said materials in a sulphide bath by an azo-dyestuff containing at least one group  $S_n$ , in which  $n$  equals 2 or 3 at a temperature lower than 65° C.

8. A process of dyeing materials which comprises treating said materials in a sulphide bath by an azo-dyestuff containing one disulphide group in the molecule, at a temperature lower than 65° C.

9. A process of dyeing materials which comprises treating said materials in a sulphide bath by an azo-dyestuff resulting from the coupling of a diazotized ortho amino phenol with an azo-component containing at least one disulphide group in the molecule, at a temperature lower than 65° C.

10. A process of dyeing materials which comprises treating said materials in a sulphide bath by an azo-dyestuff containing two disulphide groups in the molecule, at a temperature lower than 65° C.

ROBERT LANTZ.